

## UNITED STATES PATENT OFFICE

2,683,686

## METHOD OF MANUFACTURING COPPER-LEAD ALLOY COATED GRAPHITE POWDER

Tatsuo Matsukawa, Asahiku, Osaka, Japan

No Drawing. Application March 4, 1952,  
Serial No. 274,823

2 Claims. (Cl. 204—23)

1

This invention relates to the method of manufacturing copper-lead alloy coated graphite powder which is prepared by agitating the mixture of powder of zinc base alloy containing lead and that of graphite in the aqueous solution of copper salt added to them, and which is applied to materials suitable for the sintered alloy used as metal-graphite electrical brush, self-lubricating bearing metal and pantograph slider.

Materials used in the sliding part such as those above mentioned are usually manufactured by sintering copper and graphite powder, and especially, in addition to those, lead powder to reduce frictional affect. But, since these powders differ in their form and specific gravity individually, it is so difficult to mix them uniformly that a special technique is required to obtain the uniform product.

The following technique to distribute copper and graphite uniformly has been invented by the author and is described in detail in the specifications of Japanese Patents Nos. 175,387, 176,971 and 184,994. That is to coat graphite powder with copper by agitating the mixture of powder of zinc, iron or copper-zinc alloy (0.5—25% copper and zinc as balance), and that of graphite in the aqueous solution of copper sulphate or copper chloride poured onto them.

This invention proves, after the later research, that the graphite powder is able to be coated with copper-lead alloy by washing and drying the product which is obtained by agitating the mixture of powder of zinc base alloy including lead and that of graphite in the aqueous solution of copper salt added to them.

In this invention, the powder of zinc base alloy including lead, above mentioned, means as follows:

(1) Copper-lead-zinc alloy powder (in which lead is 0.5—10%, copper 0.5—20% and zinc as balance).

(2) Lead zinc alloy powder (lead 0.5—10% and zinc for the rest).

A grain size of 80—200 mesh grade is considered suitable.

With regard to the aqueous solution of copper salt, that of copper sulphate or copper chloride is preferred, but that of copper acetate or other copper salt is also available.

When the aqueous solution of copper salt is added to the mixture of powder of zinc base alloy containing lead and that of graphite, the alloy powder forms a galvanic cell with the graphite powder owing to dissolution of zinc. And the copper in the solution is deposited on the surface of cathodic powder of graphite.

Some of the fine powder of lead, resulting from decomposition of the alloy powder, is em-

2

braced mechanically in the deposited structure of copper, and, in the product, the graphite powder is coated with the mixed structure of copper and lead. And the rest of the lead powder is as well coated with deposited copper as the graphite powder.

Besides the coated powders above mentioned, fine powder of copper which does not adhere to the surface of graphite or lead powder coexists with them.

Metal graphite electrical brush, self-lubricating bearing metal or pantograph slider, manufactured by means of powder metallurgy using the kind of coated powder above described, have excellent characteristics with smaller values in their coefficients of friction and less obliteration.

A few examples in practical application of this invention are as follows:

## Example 1

1,040 cc. of aqueous solution of copper sulphate (containing 0.05 g. of copper in 1 cc. of the solution) is poured into a mixture of 65 g. of copper-lead-zinc alloy powder (the composition is 15% copper, 5% lead and 80% zinc, and the grade of powder is below 120 mesh) and 35 g. of graphite powder (below 150 mesh grade), and stirred up. After the depositing reaction of copper is over, the product is washed and dried.

## Example 2

1,384 cc. of aqueous solution of copper sulphate (containing 0.05 g. of copper in 1 cc. of the solution) is added to a mixture of 75 g. of lead-zinc alloy powder (consists of 5% lead and 95% zinc, and the size of powder is below 120 mesh grade) and 25 g. of graphite powder (below 150 mesh grade), and stirred up. After the depositing reaction of copper is concluded, the powder is washed and dried.

To illustrate the distributed state of lead for each size of powder in this method, the relation between grade distribution of raw graphite powder applied in the first example and that of produced powder of graphite coated with copper-lead alloy, and as well the contents of lead and graphite in the latter, are shown in the following table.

| 50                                                            | Size of powder, in mesh                                       | 150—200 | 200—250 | —250 |
|---------------------------------------------------------------|---------------------------------------------------------------|---------|---------|------|
| Grade distribution of raw graphite powder applied, in percent | 5                                                             | 17      | 78      |      |
| Grade distribution of coated powder produced, in percent      | 22                                                            | 24      | 54      |      |
| 55                                                            | Contents of lead in each grade of the product, in percent     | 4.10    | 3.76    | 3.32 |
|                                                               | Contents of graphite in each grade of the product, in percent | 40.3    | 39.7    | 27.9 |

The table shows that the product is larger in size than the raw graphite powder due to the coating of copper-lead alloy, and the contents of lead in every grade of powder is nearly equal. It proves that the graphite powder is able to be coated with copper-lead alloy of uniform structure by this method invented by the author.

While one illustrative embodiment of the invention has been described in detail, it is not my intention to limit its scope to that embodiment or otherwise than by the terms of the appended claims.

Having now described my invention, what I claim as new and desire to secure by Letters Patent is:

1. A process of coating graphite powder with a copper-lead alloy which comprises agitating in an aqueous solution of a copper salt the graphite powder in admixture with a lead-zinc alloy powder consisting of 0.5 to 10% lead, and the remainder zinc.

2. A process of coating graphite powder with a copper-lead alloy which comprises agitating in an aqueous solution of a copper salt the graphite powder in admixture with a lead-zinc-copper alloy powder consisting of 0.5 to 10% lead, 0.5 to 20% copper, and the remainder zinc.

References Cited in the file of this patent

UNITED STATES PATENTS

|    | Number    | Name     | Date          |
|----|-----------|----------|---------------|
| 10 | Re. 5,044 | Knight   | Aug. 27, 1872 |
|    | 20,353    | Knight   | May 25, 1858  |
|    | 901,965   | Harrison | Oct. 27, 1908 |
| 15 | 901,966   | Harrison | Oct. 27, 1908 |
|    | 1,582,617 | Mohn     | Apr. 27, 1926 |
|    | 2,414,514 | Elsey    | Jan. 21, 1947 |

OTHER REFERENCES

20 Chemical Abstracts, vol. 45, No. 19 (Oct. 20, 1951), pp. 8421-2.